

May 12, 1959

H. BERGER ET AL

2,886,726

TARGET FOR X-RADIATION AND THE LIKE

Filed Nov. 21, 1957

*Fig. 1*



*Fig. 2*



*Fig. 3*



*Fig. 4*

INVENTORS  
JOHN E. JACOBS  
HAROLD BERGER

BY

wheeler, wheeler + wheeler  
ATTORNEYS

1

2,886,726

## TARGET FOR X-RADIATION AND THE LIKE

Harold Berger, West Allis, and John E. Jacobs, Hales Corners, Wis., assignors to General Electric Company, a corporation of New York

Application November 21, 1957, Serial No. 697,823

9 Claims. (Cl. 313—65)

This invention relates to an improved target for X-radiation and the like rendered photoconductive and capable of use in apparatus to produce sharp X-ray images even though the objects from which the images are formed are moving at a relatively high rate. The invention is further concerned with a method for producing such a target.

In previously known devices of this type, lead oxide photoconductive material has been applied to a substrate material such as aluminum, aluminum being capable of good X-ray transmission. (75 Electrical Engineering 158-61, February 1956.) However, the oxide of aluminum has very high electrical resistance and the processing techniques which we desire to use have been such as to produce in a non-uniform formation of aluminum oxide between the substrate and the lead oxide coating, resulting in undesirable variation of photoconductivity characteristics from point to point.

The present invention seeks to improve the target by use of a substrate which has at least its surface composed of stainless steel or one of a number of other metal whose oxides have electrical resistance of the order of  $10^6$  ohm-cm. or less, a good degree of electrical conductivity between the substrate surface and the lead oxide being assured, and uniformity enhanced.

The substrate desirably comprises a heavy metal relatively opaque to X-radiation, whereby to filter out soft scattered radiation and produce sharper images than are otherwise obtainable. Moreover, the heavy metal intensifies the photoconductive signal by means of photo-emission from the substrate material, particularly at high X-ray energy in excess of 100 kvp. Stainless steel is ideal, but it is necessary to select an alloy having a co-efficient of expansion sufficiently close to that of the coating to preclude peeling. AISI type 430 is the most suitable alloy presently known. Since a form-sustaining sheet of stainless steel is quite opaque to X-ray, the preferred embodiments of the invention are made by electroplating or otherwise coating with a thin film of stainless steel a base plate of aluminum or other light metal which is a good electrical conductor and not unduly X-ray opaque. We have also used coatings essentially comprising copper, nickel or chromium or alloys thereof. However, stainless steel is preferred, particularly in medical applications.

Upon the substrate, lead oxide vapor is condensed and subsequently baked to convert it to a yellow crystalline form of lead oxide. The baking will oxidize the heavy metal face of the substrate at the interface and it is important that the oxide of the substrate metal should have a resistance much less than that of the lead oxide and desirably not exceeding  $10^6$  ohm-cm.

The bond between the substrate material and the lead oxide should be capable of withstanding air bake temperatures up to 700° C. for a period of several hours without melting or sagging. Its co-efficient of expansion should match that of the lead oxide sufficiently so that there will be no peeling of the lead oxide layer. The substrates herein disclosed have all of these properties and, additionally, are easily worked, relatively non-

2

magnetic, and have good X-ray transmission. Additionally, the preferred stainless steel substrate facing in particular is sufficiently heavy to act as an electron intensifier. The target plate area has been found to be notably free of the spots or blemishes found in prior target plates of this type.

In the drawings:

Fig. 1 is a diagrammatic view showing a greatly enlarged fragmentary cross section of a target embodying the invention.

Fig. 2 is a diagrammatic view showing in greatly enlarged fragmentary cross section a preferred embodiment of a target incorporating the invention.

Fig. 3 is a flow diagram of steps of the preferred method for producing a target as shown in Fig. 2.

Fig. 4 is a diagrammatic view showing in cross section apparatus used to coat the substrate with lead oxide.

In Fig. 1, the substrate 5 comprises a sheet of stainless steel or chromium or nickel of just sufficient thickness to be form sustaining. Upon this is a layer 6 of an oxide of the metal of sheet 5 and a photoconductive deposit 7 of yellow crystalline lead oxide.

In the embodiment of Fig. 2, the substrate supporting sheet 8 is aluminum or other lightweight electrically conductive metal upon which is bonded a thin deposit 50 of stainless steel preferably produced by plating or spraying it upon the substrate ply, as it is usually too thin to be self supporting. Heavier plies may be laminated to the sheet 8 by rolling. Upon the facing 50 is an oxide coating 60 on which the lead oxide layer or layers 9 and 10 are applied.

As already indicated, copper, nickel or chromium may be used in lieu of stainless steel to provide a substrate surface in lieu of the stainless steel 5 of Fig. 1 or 8 of Fig. 2. Whatever the metallic sheet or film used in the substrate to provide an interface with the lead oxide, it should be of such a nature that the oxide formed at the surface and contacted by the lead oxide should have electrical resistance very materially less than that of the lead oxide (which is  $10^{11}$  ohm-cm.). It has been found satisfactory to use as the interface portion of the substrate a metal whose oxide has a resistance of the order of  $10^6$  ohm-cm. or less. This insures proper electrical conductivity between the substrate and the deposit of lead oxide and gives results greatly superior to those achieved when the lead oxide is in contact with aluminum oxide or the like, the aluminum oxide having resistance greater than that of the lead oxide.

While the generic concept permits the use of a substrate sheet or surface film of copper, nickel or chromium, stainless steel, AISI type 430, is the preferred material used at 5 in Fig. 1 and 8 in Fig. 2 to provide the substrate surface. AISI type 430 is a preferred example principally because its co-efficient of expansion so nearly matches that of lead oxide that no separation occurs during heating or coating.

As applied, the lead oxide contains a large percentage of the red form of lead oxide. It has been found that the yellow crystalline lead oxide gives faster response to X-radiation than the red form of lead oxide. The preferred method of applying the photo-conductive layer and its conversion to the desired yellow crystalline form of lead oxide is as follows, reference being made to Fig. 3.

The substrate plate generically designated by reference character 12 may comprise the sheet 5 of Fig. 1 or the supporting sheet 8 and surface film 50 of Fig. 2. The plate 12 is placed in a vacuum chamber 13 and over it is placed a heater 14 of the electrical resistance type having current supply leads 15 and 16. Gas is thereupon withdrawn from the chamber 13 through the pipe 17

until the chamber has been evacuated. While the degree of vacuum is not critical, it has been found appropriate to draw a vacuum of 10-4 mm. Hg to 10-5 mm. Hg. Dry oxygen is then introduced through the pipe 18 in such manner as to maintain a pressure of 3 to 5 microns within the chamber. After the oxygen pressure has remained stable for 5 to 10 minutes, the substrate heater 14 is energized and the target plate 12 is raised thereby to a temperature of 360° to 380° C. This temperature is allowed to stabilize for about 30 minutes before the coating operation is commenced.

The lead oxide coating material is placed in a crucible 20 and arrangement is made for heating it by induction through the energization of the coil 21. The crucible temperature is raised slowly over a period of 10 to 20 minutes. At 830° C., the lead oxide commences to vaporize. Desirably the temperature is raised to a maximum of about 980° C., which is maintained for approximately 5 minutes. The induction heater 21 is then de-energized and the target plate 12 is allowed to cool gradually in the oxygen atmosphere for about 30 minutes. Thereupon the chamber 13 is opened by removing its cover 22 and when the target plate 12 is removed, it will have a velvety appearing red oxide coating of a red orange color and composed of a random orientation of red and yellow crystals. The target is placed immediately in a 600° C. oven and baked in air for about 90 minutes. The lead oxide is thereby converted to the yellow crystalline form.

Desirably the target is then replaced in the vacuum chamber 13, the cover 22 is sealed over it, and the coating operation is repeated to provide a second layer of lead oxide as shown at 10 in Fig. 2. The procedure is identical with that above described, including baking in air for about 90 minutes after removal of the target plate from the vacuum chamber.

The combined thickness of the two layers 9 and 10 of lead oxide is of the approximate order of 0.2 mm. and the color, in consequence of the air bake, is now yellow. The yellow crystalline lead oxide has a resistance of 10<sup>11</sup> ohm-cm. and gives a faster response to X-radiation than the red form.

During the condensation of the lead oxide on the substrate 12 in chamber 13, it is important to maintain a substrate temperature of 200° C. or greater, 350° C. or greater being preferred to get optimum results. At lower substrate or target plate temperatures, the resistivity of the lead oxide coating is lower and the image decay time is higher. The latter is particularly important, as there is a pronounced reduction in decay time as the substrate temperature during lead oxide deposit is increased to and above 200° C. A reduced decay time reduces blurring and facilitates X-ray observation of moving objects.

The baking of the lead oxide and its conversion to the yellow crystalline form necessarily results in the oxidation of the substrate material at the interface. Consequently it is important that the selected substrate metals be metals whose oxides are so formed as to provide the desired uniformity of distribution and have the desired relatively high electrical conductivity, whereby to achieve the objectives of the present invention.

The oxides of the components of the stainless steel alloy, and the metals suggested as alternatives for use in the substrate, all have resistance below the desired maximum of 10<sup>6</sup> ohm-cm. Moreover, the oxides show a uniformity of resistance throughout the interface markedly superior to that found in the oxides of the aluminum surfaces heretofore employed to support the lead oxide. Thus, blemishes and spots such as result from variations in relative conductivity in previously known targets are wholly or substantially eliminated.

The faster and higher response of the yellow lead oxide to X-radiation, in combination with the constant relative conductivity at the interface produces sharper images, and particularly unblurred images of moving objects, 75

Images are less persistent and blurring of images of moving objects is eliminated or greatly reduced. Moreover, the images are intensified by photo emission from the substrate as pointed out above.

We claim:

1. A target for converting X-radiation into an electrical signal by means of photo-conductivity and comprising a substrate plate of electrically conductive metal having a face portion and a photoconductive layer of lead oxide adherent to said face portion, the electrical conductivity of the said face portion being greatly in excess of the conductivity of the photoconductive layer.
2. A target as set forth in claim 1 in which the face portion is uniformly oxidized and comprises a metal selected from a group which includes stainless steel, chromium, nickel and copper, and the lead oxide comprises a yellow crystalline oxide of lead.
3. In a target for converting X-radiation into photoconductive action, a support plate comprising relatively light metal of self-supporting thickness and good electrical conductivity having stainless steel bonded to one of its faces in a layer too thin to be self-supporting in use, and a layer of lead oxide on an exposed face of the stainless steel and forming a photoconductor, the coefficient of thermal expansion of the lead oxide and the stainless steel being so nearly identical as to avoid cracking off the lead oxide in the course of changes of temperature affecting the target.
4. In a target for converting X-radiation into photoconductive action, a plate providing mechanical support and comprising relatively light metal of good electrical conductivity, said plate having a facial coating of a heavier metal uniformly superficially oxidized, and a layer of photoconductive yellow lead oxide on the superficial oxide of heavier metal, the oxide of the heavy coating metal becoming very substantially more conductive electrically than the yellow lead oxide and having approximately the same co-efficient of thermal expansion, relative conductivity of the oxidized surface of the heavier metal coating and the oxide being substantially uniform throughout the interface therebetween.
5. The target of claim 4 in which the coating of heavier metal is less conductive to X-radiation than the support plate and filters soft and scattered rays of X-radiation, thereby intensifying the photoconductive response of the yellow lead oxide layer when the target is subjected to X-radiation.
6. The target defined in claim 5 in which the coating metal is selected from the group consisting of stainless steel, copper, nickel, chromium and alloys of steel, copper, nickel or chromium.
7. The target of claim 5 in which the coating metal comprises stainless steel of the type defined as AISI type 430.
8. The method of making a target plate for converting X-radiation into photo-conductive action, which method comprises plating a substrate of lightweight and self-sustaining thickness and capable of good X-ray transmission with a ply of materially heavier metal to a thickness inadequate for self-support, whereby the plated ply is dependent on the substrate for support, and subsequently applying lead oxide to the surface of said ply, and baking the substrate and said ply and coating, producing an oxide on the said ply which has materially greater electrical conductivity than the lead oxide, and concurrently converting the lead oxide to yellow lead oxide.
9. The method recited in claim 8 in which said ply comprises stainless steel.

References Cited in the file of this patent

UNITED STATES PATENTS

|           |                    |               |
|-----------|--------------------|---------------|
| 2,169,840 | Lewis et al. ----- | Aug. 15, 1939 |
| 2,747,132 | Sheldon -----      | May 22, 1956  |

UNITED STATES PATENT OFFICE  
CERTIFICATE OF CORRECTION

Patent No. 2,886,726

May 12, 1959

Harold Berger et al.

It is hereby certified that error appears in the printed specification of the above numbered patent requiring correction and that the said Letters Patent should read as corrected below.

Column 4, line 36, for "becoming" read -- being --.

Signed and sealed this 15th day of September 1959.

(SEAL)

Attest:

KARL H. AXLINE  
Attesting Officer

ROBERT C. WATSON  
Commissioner of Patents